

# United States Patent [19]

Olson et al.

[11] Patent Number: 5,006,126

[45] Date of Patent: Apr. 9, 1991

[54] **CELLULASE COMPOSITIONS AND METHODS THAT INTRODUCE VARIATIONS IN COLOR DENSITY INTO CELLULOSIC FABRICS, PARTICULARLY INDIGO DYED DENIM**

[75] Inventors: **Lynne A. Olson, Mendota Heights; Patricia M. Stanley, Minneapolis, both of Minn.**

[73] Assignee: **Ecolab Inc., St. Paul, Minn.**

[21] Appl. No.: **245,123**

[22] Filed: **Sep. 15, 1988**

[51] Int. Cl.<sup>5</sup> ..... **C11D 3/38; C11D 11/00; D06B 11/00**

[52] U.S. Cl. ..... **8/401; 8/653; 8/918; 252/8.6; 252/8.8; 252/8.9**

[58] **Field of Search** ..... **8/401; 252/8.8, 8.9**

[56] **References Cited**

**U.S. PATENT DOCUMENTS**

4,435,307 3/1984 Barbesgaard ..... 252/174.12  
4,443,355 4/1984 Murata et al. ..... 252/174.12  
4,479,881 10/1984 Tai ..... 252/8.8

4,661,289 4/1987 Parslow et al. ..... 252/8.8  
4,832,864 5/1989 Olson ..... 252/174.12  
4,912,056 3/1990 Olson ..... 8/116.1

*Primary Examiner*—A. Lionel Clingman  
*Attorney, Agent, or Firm*—Merchant, Gould, Smith, Edell, Welter & Schmidt

[57] **ABSTRACT**

Aqueous processes and compositions of the invention for obtaining a "stone-washed", distressed or "used and abused" look in clothing, particularly in the panels and seams of denim jeans and jackets involve compositions that are stone-free that avoid mechanical abrasion of the fabric. In particular, the process and composition of the invention used to obtain the distressed, "stone-washed" or "acid washed look" are free of common pumice or pumice-bleach compositions, used in large institutional-size laundry machines, and rely solely on the chemical action of aqueous treatment compositions. The aqueous treatments can be made from liquid or solid concentrates.

**9 Claims, 1 Drawing Sheet**

• • • • • • • • • **PRODUCT OF EXAM. II**

— — — — — **STANDARD STONE-  
WASHED JEANS**



• • • • • PRODUCT OF EXAM. II

— — — — — STANDARD STONE-  
WASHED JEANS



**CELLULASE COMPOSITIONS AND METHODS  
THAT INTRODUCE VARIATIONS IN COLOR  
DENSITY INTO CELLULOSIC FABRICS,  
PARTICULARLY INDIGO DYED DENIM**

**FIELD OF THE INVENTION**

The invention relates to the manufacture of clothing from dyed cellulosic fabrics. More particularly, the invention relates to pumice-free compositions and processes used in the manufacture of a clothing item, preferably from denim fabric dyed with indigo, that can produce in a clothing item a distressed, "used and abused" appearance that is virtually indistinguishable from the appearance of "stone washed" clothing items made by traditional pumice processing.

**BACKGROUND OF THE INVENTION**

Clothing made from cellulosic fabrics such as cotton and in particular indigo dyed denim fabrics have been common items of clothing for many years. Such clothing items are typically sold after they are sewn from sized and cut cloth. Such clothes and particularly denim clothing items are stiff in texture due to the presence of sizing compositions used to ease manufacturing, handling and assembling of the clothing items and typically have a fresh dark dyed appearance. After a period of wear, the clothing items, particularly denim, can develop in the clothing panels and on seams, localized areas of variations, in the form of a lightening, in the depth or density of color. In addition a general fading of the clothes can often appear in conjunction with the production of a "fuzzy" surface, some pucker in seams and some wrinkling in the fabric panels. Additionally, after laundering, sizing is substantially removed from the fabric resulting in a softer feel. In recent years such a distressed or "used and abused" look has become very desirable, particularly in denim clothing, to a substantial proportion of the public. To some extent, a limited pre-worn appearance, which has a uniform color density different than the variable color density in the typical stone-washed item, can be produced through pre-washing or preshrinking processes.

The preferred methods for producing the distressed "used and abused" look involve stone washing of a clothing item. Stone washing comprises contacting a denim clothing item or items in large tub equipment with pumice stones having a particle size of about 1 to 10 inches and with smaller pumice particles generated by the abrasive nature of the process. Typically the clothing item is tumbled with the pumice while wet for a sufficient period such that the pumice abrades the fabric to produce in the fabric panels, localized abraded areas of lighter color and similar lightened areas in the seams. Additionally the pumice softens the fabric and produces a fuzzy surface similar to that produced by the extended wear of the fabric.

The 1 to 10 inch pumice stones and particulate pumice abrasion by-products can cause significant processing and equipment problems. Particulate pumice must manually be removed from processed clothing items (de-rocking) because they tend to accumulate in pockets, on interior surfaces, in creases and in folds. In the stone washing machine, the stones can cause overload damage to electric motors, mechanical damage to transport mechanisms and washing drums and can significantly increase the requirements for machine maintenance. The pumice stones and particulate material can

clog machine drainage passages and can clog drains and sewer lines at the machine site. Further, the abraded pumice can clog municipal sewer lines, can damage sewage processing equipment, and can significantly increase maintenance required in municipal sewage treatment plants. These problems can add significantly to the cost of doing business and to the purchase price of the goods.

In view of the problems of pumice in stone washing, increasing attention has been directed to finding a replacement for stone washing in garment manufacture (see the Wall Street Journal, May 27, 1987, p. 1.). One avenue of investigation involves using a replacement stone such as a synthetic abrasive. In particular, ceramic balls such as those used in ball mills and irregular hard rubber pieces, which can be used without producing abraded by-products, have been experimented with in stone washing processes. These materials reduce the unwanted effects caused by particulate by-product pumice but do not significantly reduce machine damage caused by stones or the required maintenance on stone-containing laundry tubs. As a result, significant attention has been directed to producing a stone-free or pumice-free "stone washed" process that can produce a stone-washed denim look.

One disadvantage in pumice processing is that pumice cannot be used in tunnel washers, the largest commercial washing machines. Pumice cannot be circulated through the tunnel machines due to machine internal geometry. The use of larger-scale tunnel washers could significantly increase the productivity of the processes with the use of a stone or pumice-free composition that produces a genuine "stone-washed" look.

Barbesgarrd et al, U.S. Pat. No. 4,435,307 teach a specific cellulase enzyme that can be obtained from *Humicola insolens* which can be used in soil removing detergent compositions. Martin et al, European Pat. Application No. 177,165 teach fabric washing compositions containing a surfactant, builders, and bleaches in combination with a cellulase composition and a clay, particularly a smectite clay. Murata et al, U.K. Pat. Application No. 2,095,275 teach enzyme containing detergent compositions comprising an alkali cellulase and typical detergent compositions in a fully formulated laundry preparation. Tai, U.S. Pat. No. 4,479,881 teaches an improved laundry detergent containing a cellulase enzyme in combination with a tertiary amine in a laundry preparation. Murata et al, U.S. Pat. No. 4,443,355 teach laundry compositions containing a cellulase from a *cellulosmonas* bacteria. Parslow et al, U.S. Pat. No. 4,661,289 teaches fabric washing and softening compositions containing a cationic softening agent and a fungal cellulase in conjunction with other typical laundry ingredients. Suzuki, U.K. Pat. Application No. 2,094,826 teaches detergent laundry compositions containing a cellulase enzyme.

dyed cellulosic clothing (such as denim) have been treated with desizing enzymes, detergents, bleaches, sours and softeners in prewashing and preshrinking processes. These variations are not intended to and do not duplicate the "stone-washed" look. A stone or pumice-free "stone-washed" process that produces the true stone-washed look has yet to be developed.

**BRIEF DESCRIPTION OF THE INVENTION**

We have found that the "stone washed" appearance that takes the form of variations in local color density in

fabric panels and seams of dyed cellulosic fabric, particularly in denim, clothing items can be substantially obtained using a stone or pumice-free process in which the clothing items are mechanically agitated in a tub with an aqueous composition containing amounts of a cellulase enzyme that can degrade the cellulosic fabric and can release the fabric dye or dyes.

The aqueous treatment compositions are obtained by diluting a novel "stone-wash" liquid or solid concentrate consisting essentially of a cellulase enzyme and a diluent such as a compatible surfactant composition, a non-aqueous solvent or a solid-forming agent capable of suspending the cellulase without significant loss of enzymatic activity.

The use of cellulase enzyme preparations is known in laundry cleaning or detergent compositions. Such detergent compositions that are designed for soil removal typically contain surfactants (typically anionic), fillers, brighteners, clays, cellulase and other enzymes (typically proteases, lipases or amylases) and other laundry components to provide a full functioning laundry detergent preparation. The cellulase enzymes in such laundry preparations are typically used (at a concentration less than 500 to 900 CMC units per liter of wash liquor) for the purpose of removing surface fibrils or particles produced by fabric wear which tend to give the fabric a used or faded appearance. The cellulase enzymes in combination with the surfactants used in common laundry compositions for cleaning apparently can remove particulate soil and can restore the new appearance of clothing items. Such compositions are not known to introduce, into clothing, areas of variation in color density which can generally be undesirable in the laundry processing.

For the purpose of this invention, the terms stone-washed appearance and variations in local color depth or density in fabric materials are synonymous. The stone-washed appearance is produced in standard processing in fabric through an abrasion process wherein pumice apparently removes surface bound dye in a relatively small portion of the surface of a garment. Such an abraded area varies from the surrounding color or depth density and is substantially lighter in color. The production of such relatively small local areas of lightness or variation in color depth or density is the goal of both pumice containing stone washing processes in the prior art and Applicant's stone-free chemical treatment methods and compositions.

#### BRIEF DESCRIPTION OF DRAWINGS

FIG. 1 is a graph demonstrating the similarity in visual spectrophotometric character of authentic stone-washed jeans when compared to jeans produced by the compositions and methods of the invention.

#### DETAILED DESCRIPTION OF THE INVENTION

The stone free "stone washed" methods of the invention involve contacting clothing items or denim fabric with an aqueous solution containing a cellulase enzyme composition and agitating the treated fabric for a sufficient period of time to produce localized variations in color density in the fabric. The fabric items can be wet by the solution and agitated apart from the bulk aqueous liquors or can be agitated in the liquor. Typically the aqueous solution contains the cellulase enzyme and a cellulase compatible surfactant that increases the wet-

ting properties of the aqueous solution to enhance the cellulase effect.

The aqueous treatment solutions are typically prepared from a liquid or solid concentrate composition which can be diluted with water at appropriate dilution ratios to formulate the aqueous treatment. The "stone wash concentrate" compositions typically contain the cellulase enzyme and a diluent such as a compatible surfactant, a nonaqueous solvent or a solid-forming agent that can produce in a treatment liquor a suspension of the cellulose enzyme without significant enzyme activity loss.

The solid concentrate compositions typically comprise a suspension of the cellulase enzyme composition in a solid matrix. The solid matrixes can be inorganic or organic in nature. The solid concentrates can take the form of large masses of solid concentrate or can take the form of granular or pelletized composition. The solid concentrates can be used in commercial processes by placing the solid concentrate materials in dispensers that can direct a dissolving spray of water onto the solid or pellet material thereby creating a concentrated solution of the material in water which is then directed by the dispenser into the wash liquors contained in the commercial drum machines.

#### CELLULASE ENZYME

Enzymes are a group of proteins which catalyze a variety of typically biochemical reactions. Enzyme preparations have been obtained from natural sources and have been adapted for a variety of chemical applications. Enzymes are typically classified based on the substrate target of the enzymatic action. The enzymes useful in the compositions of this invention involve cellulase enzymes (classified as I.U.B. No. 3.2.1.4., EC numbering 1978). Cellulase are enzymes that degrade cellulose by attacking the C(1→4) (typically beta) glucosidic linkages between repeating units of glucose moieties in polymeric cellulosic materials. The substrate for cellulase is cellulose, and cellulose derivatives, which is a high molecular weight natural polymer made of polymerized glucose. Cellulose is the major structural polymer of plant organisms. Additionally cellulose is the major structural component of a number of fibers used to produce fabrics including cotton, linen, jute, rayon and ramie, and others.

Cellulases are typically produced from bacterial and fungal sources which use cellulase in the degradation of cellulose to obtain an energy source or to obtain a source of structure during their life cycle. Examples of bacteria and fungi which produce cellulase are as follows: *Bacillus hydrolyticus*, *Cellulobacillus mucosus*, *cellulobacillus myxogenes*, *Cellulomonas* sp., *Cellvibrio fulvus*, *Cellvibrio vulgaris*, *Clostridium thermocellulaseum*, *Clostridium thermocellum*, *Corynebacterium* sp., *Cytophaga globulosa*, *Pseudomonas fluoroescens* var. *cellulosa*, *Pseudomonas solanacearum*, *Bacterioides succinogenes*, *Ruminococcus albus*, *Ruminococcus flavefaciens*, *Soran-dium* composition, *Butyrivibrio*, *Clostridium* sp., *Xanthomonas cymopsidis*, *Sclerotium bataticola*, *Bacillus* sp., *Thermoactinomyces* sp., *Actinobifida* sp., *Actinomycetes* sp., *Streptomyces* sp., *Arthrobotrys superba*, *Aspergillus aureus*, *Aspergillus flavipes*, *Aspergillus flavus*, *Aspergillus fumigatus*, *Aspergillus fuchuenis*, *Aspergillus nidulans*, *Aspergillus niger*, *Aspergillus oryzae*, *Aspergillus rugulosus*, *Aspergillus sojae*, *Aspergillus sydwi*, *Aspergillus tamaril*, *Aspergillus terreus*, *Aspergillus unguis*, *Aspergillus ustus*, *Takamine-Cellulase*, *Aspergillus saitoi*, *Botrytis*

*cinerea*, *Botryodipiodia theobromae*, *Cladosporium cucumerinum*, *Cladosporium herbarum*, *Coccospora agricola*, *Curvularia lunata*, *Chaetomium thermophile* var. *coprophile*, *Chaetomium thermophile* var. *dissitum*, *Sporotrichum thermophile*, *Taromycetes amersonii*, *Thermoascus aurantiacus*, *Humicola grisea* var. *thermoidea*, *Humicola insolens*, *Malbrancheda puicella* var. *sulfurea*, *Myriococcum albomyces*, *Stilbella thermophile*, *Torula thermophila*, *Chaetomium globosum*, *Dictyostelium discoideum*, *Fusarium* sp., *Fusarium bulbigenum*, *Fusarium equiseti*, *Fusarium lateritium*, *Fusarium lini*, *Fusarium oxysporum*, *Fusarium vasicinectum*, *Fusarium dimerum*, *Fusarium japonicum*, *Fusarium scirpi*, *Fusarium solani*, *Fusarium moniliforme*, *Fusarium roseum*, *Helminthosporium* sp., *Memnoniella echinata*, *Humicola fucoatra*, *Humicola grisea*, *Monilia sitophila*, *Monosporopsis brevis*, *Mucor pusillus*, *Mycosphaerella citrulina*, *Myrothecium verrucaria*, *Papulaspore* sp., *Penicillium* sp., *Penicillium capsulatum*, *Penicillium chrysogenum*, *Penicillium frequentana*, *Penicillium funiculosum*, *Penicillium janthinellum*, *Penicillium luteum*, *Penicillium piscarium*, *Penicillium soppi*, *Penicillium spinulosum*, *Penicillium turbaturn*, *Penicillium digitatum*, *Penicillium expansum*, *Penicillium pusillum*, *Penicillium rubrum*, *Penicillium wortmanii*, *Penicillium variabile*, *Pestalotia palmarum*, *Pestalotiopsis westerdijkii*, *Phoma* sp., *Schizophyllum commune*, *Scopulariopsis brevicaulis*, *Rhizopus* sp., *Sporotrichum carnis*, *Sporotrichum pruinosa*, *Stachybotrys atra*, *Torula* sp., *Trichoderma viride* (reesei), *Trichurus cylindricus*, *Verticillium albo atrum*, *Aspergillus celulosa*, *Penicillium glaucum*, *Cunninghamella* sp., *Mucor mucedo*, *Rhizopus chinensis*, *Coremiella* sp., *Karlingia rosea*, *Phytophthora cactorum*, *Phytophthora citricola*, *Phytophthora parasitica*, *Pythium* sp., *Saprolegniaceae*, *Ceratocystis ulmi*, *Chaetomium globosum*, *Chaetomium indicum*, *Neurospora crassa*, *Sclerotium rolfsii*, *Aspergillus* sp., *Chrysosporium lignorum*, *Penicillium notatum*, *Pyricularia oryzae*, *Collybia velutipes*, *Coprinus sclerotigenus*, *Hydnus henningsii*, *Irpea lactea*, *Polyporus sulphureus*, *Polyporus betreus*, *Polystictus hirsutus*, *Trametes vitata*, *Irpea consolus*, *Lentipes lepidus*, *Poria vaporaria*, *Fomes pinicola*, *Lenzites styracina*, *Merulius lacrimans*, *Polyporus palustris*, *Polyporus annosus*, *Polyporus versicolor*, *Polystictus sanguineus*, *Poris vailantii*, *Puccinia graminis*, *Tricholome fumosum*, *Tricholome nudum*, *Trametes sanguinea*, *Polyporus schweinitzii* FR., *Conidio-phora carebella*, *Cellulase AP* (Amano Pharmaceutical Co., Ltd.), *Cellulosin AP* (Ueda Chemical Co., Ltd.), *Cellulosin AC* (Ueda Chemical Co., Ltd.), *Cellulase-Onozuka* (Kinki Yakult Seizo Co., Ltd.), *Pancellase* (Kinki Yakult Seizo Co., Ltd.), *Macerozyme* (Kinki Yakult Seizo Co., Ltd.), *Meicelase* (Meiji Selka Kaisha, Ltd.), *Celluzyme* (Nagase Co., Ltd.), *Soluble cellulase* (Sankyo Co., Ltd.), *Sanzyme* (Sankyo Co., Ltd.), *Cellulase A-12-C* (Takeda Chemical Industries, Ltd.), *Toyo-Cellulase* (Toyo Jozo Co., Ltd.), *Driserase* (Kyowa Hakko Kogyo Co., Ltd.), *Luizyme* (Luipold Werk), *Takamine-Cellulase* (Chemische Fabrik), *Wallerstein-Cellulase* (Sigma Chemicals), *Cellulase Type I* (Sigma Chemicals), *Cellulase Serva* (Serva Laboratory), *Cellulase 36* (Rohm and Haas), *Miles Cellulase 4,000* (Miles), *R & H Cellulase 35, 36, 38 conc* (Phillip Morris), *Com-bizym* (Nysco Laboratory), *Cellulase* (Makor Chemicals), *Cellulast*, *Celluzyme*, *Cellucrust* (NOVO Industry), and *Cellulase* (Gist-Brocades). *Cellulase* preparations are available from *Accurate Chemical & Scientific Corp.*, *Alltech, Inc.*, *Amano International Enzyme*, *Boehringer Mannheim Corp.*, *Calbiochem Biochems*,

Carolina Biol. Supply Co., Chem. Dynamics Corp., Enzyme Development, Div. Biddle Sawyer, Fluka Chem. Corp., Miles Laboratories, Inc., Novo Industrials (Biolabs), Plenum Diagnostics, Sigma Chem. Co., Un. States Biochem. Corp., and Weinstein Nutritional Products, Inc.

Cellulase, like many enzyme preparations, is typically produced in an impure state and often is manufactured on a support. The solid cellulase particulate product is provided with information indicating the number of international enzyme units present per each gram of material. The activity of the solid material is used to formulate the treatment compositions of this invention. Typically the commercial preparations contain from about 1,000 to 6,000 CMC enzyme units per gram of product.

## SURFACTANT

20 A surfactant can be included in the treatment compositions of the invention. The surfactant can increase the wettability of the aqueous solution promoting the activity of the cellulase enzyme in the fabric. The surfactant increases the wettability of the enzyme and fabric. The surfactant facilitates the exclusion of air bubbles from 25 fabric surfaces and the enzyme preparation, and promotes contact between enzyme and fabric surface. The properties of surfactants are derived from the presence of different functional groups.

- Surfactants are classified and well known categories including nonionic, anionic, cationic and amphoteric surfactants.

Nonionic surfactants are surfactants having no charge when dissolved or dispersed in aqueous medium. The hydrophilic tendency of nonionic surfactants is derived from oxygen typically in ether bonds which are hydrated by hydrogen bonding to water molecules. Hydrophilic moieties in nonionics can also include hydroxyl groups and ester and amide linkages. Typical nonionic surfactants include alkyl phenol alkoxylates, aliphatic alcohol alkoxylates, carboxylic acid esters, carboxylic acid amides, polyalkylene oxide heteric and block copolymers, and others.

Nonionic surfactants are generally preferred for use in the compositions of this invention since they provide the desired wetting action and do not degrade the enzyme activity. Preferred nonionic surfactants include polymeric molecules derived from repeating units of ethylene oxide, propylene oxide, or mixtures thereof. Such nonionic surfactants include both homopolymeric, heteropolymeric, and block polymeric surfactant molecules. Included within the preferred class of non-ionic surfactants are polyethylene oxide polymers, poly-propylene oxide polymers, ethylene oxide-propylene oxide block copolymers, ethoxylated C<sub>1-18</sub> alkyl phenols, ethoxylated C<sub>1-18</sub> aliphatic alcohols, pluronic surfactants, reverse pluronic surfactants, and others.

Particularly preferred nonionics include: polyoxyethylene alkyl or alkenyl ethers having alkyl or alkenyl groups of a 10 to 20 average carbon number and having 60 1 to 20 moles of ethylene oxide added; polyoxyethylene alkyl phenyl ethers having alkyl groups of a 6 to 12 average carbon number and having 1 to 20 moles of ethylene oxide added; polyoxypropylene alkyl or alkenyl ethers having alkyl groups or alkenyl groups of a 10 65 to 20 average carbon number and having 1 to 20 moles of propylene oxide added; polyoxybutylene alkyl or alkenyl ethers having alkyl groups of alkenyl groups of a 10 to 20 average carbon number and having 1 to 20

moles of butylene oxide added; nonionic surfactants having alkyl groups or alkenyl groups of a 10 to 20 average carbon number and having 1 to 30 moles in total of ethylene oxide and propylene oxide or ethylene oxide and butylene oxide added (the molar ratio of ethylene oxide to propylene oxide or butylene oxide being 0.1/9.9 to 9.9/0.1); or higher fatty acid alkanolamides or alkylene oxide adducts thereof. Less preferred surfactants include anionic, cationic and amphoteric surfactants.

Anionic surfactants are surfactants having a hydrophilic moiety in an anionic or negatively charged state in aqueous solution. Commonly available anionic surfactants include carboxylic acids, sulfonic acids, sulfuric acid esters, phosphate esters, and salts thereof.

Cationic surfactants are hydrophilic moieties wherein the charge is cationic or positive when dissolved in aqueous medium. Cationic surfactants are typically found in amine compounds, oxygen containing amines, amide compositions, and quaternary amine salts. Typical examples of these classes are primary and secondary amines, amine oxides, alkoxylated or propoxylated amines, carboxylic acid amides, alkyl benzyl dimethyl ammonium halide salts and others.

Amphoteric surfactants which contain both acidic and basic hydrophilic structures tend to be of reduced utility in most fabric treating processes.

#### SOLVENTS

Solvents that can be used in the liquid concentrate compositions of the invention are liquid products that can be used for dissolving or dispersing the enzyme and surfactant compositions of the invention. Because of the character of the preferred nonionic surfactants, the preferred solvents are oxygen containing solvents such as alcohols, esters, glycol, glycol ethers, etc. Alcohols that can be used in the composition of the invention include methanol, ethanol, isopropanol, tertiary butanol, etc. Esters that can be used include amyl acetate, butyl acetate, ethyl acetate, esters of glycols, and others. Glycols and glycol ethers that are useful as solvents in the invention include ethylene glycol, propylene glycol, and oligomers and higher polymers of ethylene or propylene glycol in the form of polyethylene or polypropylene glycols. In liquid concentrates the low molecular weight oligomers are preferred. In solid organic concentrates the high molecular weight polymers are preferred.

#### SOLID FORMING AGENTS

The compositions of the invention can be formulated in a solid form such as a cast solid, large granules or pellets. Such solid forms are typically made by combining the cellulase enzyme with a solidification agent and forming the combined material in a solid form. Both organic and inorganic solidification agents can be used. The solidification agents must be water soluble or dispersible, compatible with the cellulase enzyme, and easily used in manufacturing equipment.

Inorganic solid forming agents that can be used are typically hydratable alkali metal or alkaline earth metal inorganic salts that can solidify through hydration. Such compositions include sodium, potassium or calcium, carbonate, bicarbonate, tripolyphosphate silicate, and other hydratable salts. The organic solidification agents typically include water soluble organic polymers such as polyethylene oxide or polypropylene oxide polymers having a molecular weight of greater than

about 1,000, preferably greater than about 1,400. Other water soluble polymers can be used including polyvinyl alcohol, polyvinyl pyrrolidone, polyalkyl oxazolines, etc. The preferred solidification agent comprises a polymer of polyethylene oxide having an average molecular weight of greater than about 1,000 to about 20,000, preferably 1,200 to 10,000. Such compositions are commercially available as CARBOWAX® 1540, 4000, 6000. To the extent that the nonionic surfactants and other ingredients are soluble in solid polymer compositions, the solid organic matrices can be considered solvent.

Additionally, the solid pellet-like compositions of the invention can be made by pelletizing the enzyme using well known pressure pelletizing techniques in which the cellulase enzyme in combination with a binder is compacted under pressure to a tablet or pellet composition.

#### ALKALIS OR INORGANIC ELECTROLYTES

The composition may also contain 1-50 wt-%, preferably 5-30 wt-% of one or more alkali metal salts selected from the following compounds as the alkali or inorganic electrolyte: silicates, carbonates and sulfates. Further, the composition may contain organic alkalis such as triethanolamine, diethanolamine, monoethanolamine, and triisopropanolamine.

#### MASKING AGENTS FOR FACTORS INHIBITING THE CELLULASE ACTIVITY

The cellulases are deactivated in some cases in the presence of heavy metal ions including copper, zinc, chromium, mercury, lead, manganese, or silver ions or their compounds. Various metal chelating agents and metal-precipitating agents are effective against these inhibitors. They include, for example, divalent metal ion sequestering agents as listed below with reference to optional additives as well as magnesium silicate and magnesium sulfate.

Cellobiose, glucose and gluconolactone can act as an inhibitor. It is preferred to avoid the co-presence of these saccharides with the cellulase if possible. In case the co-presence is unavoidable, it is necessary to avoid the direct contact of the saccharides with the cellulase by, for example, coating them.

Long chain fatty acid salts and cationic surfactants act as the inhibitors in some cases. However, the co-presence of these substances with the cellulase is allowable if the direct contact of them is prevented by some means such as tableting or coating.

The above-mentioned masking agents and methods may be employed, if necessary, in the present invention.

#### CELLULASE-ACTIVATORS

The activators vary depending on variety of the cellulases. In the presence of proteins, cobalt and its salts, magnesium and its salts, and calcium and its salts, potassium and its salts, sodium and its salts or monosaccharides such as mannose and xylose, the cellulases are activated and their deterging powers can be improved.

#### ANTIOXIDANTS

The antioxidants include, for example, tert-butylhydroxytoluene, 4,4'-butyldenebis(6-tert-butyl-3-methylphenol), 2,2'-butyldenebis(6-tert-butyl-4-methylphenol), monostyrenated cresol, distyrenated cresol, monostyrenated phenol, distyrenated phenol and 1,1-bis(4-hydroxyphenyl)cyclohexane.

## SOLUBILIZERS

The solubilizers include, for example, lower alcohols such as ethanol, benzenesulfonate salts, lower alkylbenzenesulfonate salts such as p-toluenesulfonate salts, glycols such as propylene glycol, acetylbenzenesulfonate salts, acetamides, pyridinedicarboxylic acid amides, benzoate salts and urea.

The detergent composition of the present invention can be used in a broad pH range of about 6.5 to 10, preferably 6.5 to 8.

## BUILDERS

## Divalent Sequestering Agents

The composition may contain 0-50 wt-% of one or more builder components selected from the group consisting of alkali metal salts and alkanolamine salts of the following compounds: phosphates such as orthophosphate, pyrophosphate, tripolyphosphate, metaphosphate, hexametaphosphate and phytic acid; phosphonates such as ethane-1,1-diphosphonate, ethane-1,1,2-triphosphonate, ethane-1-hydroxy-1,1-diphosphonate and its derivatives, ethanehydroxy-1,1,2-triphosphonate, ethane-1,2-dicarboxy-1,2-diphosphonate and methanehydroxyphosphonate; phosphonocarboxylates such as 2-phosphonobutane-1,2-dicarboxylate, 1-phosphonobutane-2,3,4tricarboxylate and  $\alpha$ -methylphosphonosuccinate; salts of amino acids such as aspartic acid, glutamic acid and glycine; aminopolycetates such as nitrilotriacetate, ethylenediaminetetraacetate, diethylenetriaminepentaacetate, iminodiacetate, glycol ether diamine tetraacetate, hydroxyethyliminodiacetate; high molecular electrolytes such as polyacrylic acid, polyaconitic acid, polyitaconic acid, polycitramonic acid, polyfumaric acid, polymaleic acid, polymesaconic acid, poly- $\alpha$ -hydroxyacrylic acid, polyvinylphosphonic acid, sulfonated polymaleic acid, maleic anhydride/diisobutylene copolymer, maleic anhydride/styrene copolymer, maleic anhydride/methyl vinyl ether copolymer, maleic anhydride/ethylene copolymer, maleic anhydride/ethylene crosslinked copolymer, maleic anhydride/vinyl acetate copolymer, maleic anhydride/acrylonitrile copolymer, maleic anhydride/acrylic ester copolymer, maleic anhydride/-butadiene copolymer, maleic anhydride/isoprene copolymer, poly- $\beta$ -ketocarboxylic acid derived from maleic anhydride and carbon monoxide, itaconic acid/ethylene copolymer, itaconic acid/aconic acid copolymer, itaconic acid/maleic acid copolymer, itaconic acid/acrylic acid copolymer, malonic acid/methylene copolymer, mesaconic acid/fumaric acid copolymer, ethylene glycol/ethylene terephthalate copolymer, vinylpyrrolidone/vinyl acetate copolymer, 1-butene-2,3,4-tricarboxylic acid/itaconic acid/acrylic acid copolymer, polyester polyaldehydocarboxylic acid containing quaternary ammonium group, cis-isomer of epoxysuccinic acid, poly[N,N-bis(carboxymethyl)acrylamide], poly(hydroxycarboxylic acid), starch/succinic acid or maleic acid or terephthalic acid ester, starch/phosphoric acid ester, dicarboxystarch, dicarboxymethylstarch, and cellulose/succinic acid ester; non-dissociating polymers such as polyethylene glycol, polyvinyl alcohol, polyvinyl pyrrolidone and cold water soluble, urethanated polyvinyl alcohol; and salts of dicarboxylic acids such as oxalic acid, malonic acid, succinic acid, glutaric acid, adipic acid, pimelic acid, suberic acid, azelaic acid and decane-1,10-dicarboxylic acid; salts of diglycolic acid, thioglycolic acid, oxal-

acetic acid, hydroxydisuccinic acid, carboxymethylhydroxysuccinic acid and carboxymethyltartronic acid; salts of hydroxycarboxylic acids such as glycolic acid, malic acid, hydroxypivalic acid, tartaric acid, citric acid, lactic acid, gluconic acid, mucic acid, glucuronic acid and dialdehydrostarch oxide; salts of itaconic acid, methylsuccinic acid, 3-methylglutaric acid, 2,2-dimethylmalonic acid, maleic acid, fumaric acid, glutamic acid, 1,2,3-propanetricarboxylic acid, aconitic acid, 3-butene-1,2,3-tricarboxylic acid, butane-1,2,3,4-tetracarboxylic acid, ethanetetracarboxylic acid, ethenetetracarboxylic acid, n-alkenylaconitic acid, 1,2,3,4-cyclopentanetetracarboxylic acid, phthalic acid, trimesic acid, hemimellitic acid, pyromellitic acid, benzenehexacarboxylic acid, tetrahydrofuran-1,2,3,4-tetracarboxylic acid and tetrahydrofuran-2,2,5,5-tetracarboxylic acid; salts of sulfonated carboxylic acids such as sulfoitaconic acid, sulfotricarballylic acid, cysteic acid, sulfoacetic acid and sulfosuccinic acid; carboxymethylated sucrose, lactose and raffinose, carboxymethylated pentaerythritol, carboxymethylated gluconic acid, condensates of polyhydric alcohols or sugars with maleic anhydride or succinic anhydride, condensates of hydroxycarboxylic acids with maleic anhydride or succinic anhydride, and the like.

The cellulase treatment compositions of the invention can be manufactured in the form of a thickened liquid or a gel. Common organic and inorganic compositions can be used to produce the thickened or gelled product form. Such a product form is useful in enzyme preparations wherein the enzyme tends to be salted out by the concentration of inorganic or organic buffer components. The thickened or gelled compositions tend to maintain the uniformity of the enzyme containing compositions and can ensure that the enzyme treatments are uniform. A non-uniform product can result in either large excesses of enzyme or absence of enzyme. Such thickeners include organic and naturally occurring polymers such as ethylene vinyl acetate copolymers, polyethylene waxes, acrylic polymers, cellulosic polymers including carboxymethyl cellulose, carboxyethyl cellulose, cellulose acetates, ethoxylated cellulose, alkanolamides, waxy alcohols, and others; magnesium aluminum silicates, bentonite clays, fumed silica, xanthan guar gum, algin derivatives, polyvinyl pyrrolidone, di and tristearate salts, and other conventional thickeners.

We have found that the preferred mode of contacting the dyed cellulosic fabrics with the treatment compositions of the invention is to maintain as set forth above the concentration of the enzyme in the aqueous treating solution at at least 1,000 CMC units of enzyme per liter of solution, preferably greater than 1,500 CMC units of enzyme per liter of solution. Additionally we have found that controlling the ratio between treating solution and fabric is important in optimizing the treatment. We have found that maintaining the amount of aqueous treatment to about 1 to about 10 milliliters of treatment solution per gram of fabric aids in the economic treatment of the dyed cellulosic fabrics, primarily indigo dyed denim, to obtain optimal used and abused appearance.

In somewhat greater detail, the clothing items can be contacted with an aqueous solution containing cellulase enzyme and a surfactant to promote the action of the cellulase for a sufficient time to produce local variations in color density in the surface of the fabric. The amount of solution used to treat the clothing items typically

depends on the ratio of cellulase in the product and the dry weight of the clothing items to be washed. Typically the solutions used in the methods of the invention can contain a minimum of about 6,500 CMC units of cellulase per liter, preferably 1,750 to 7,500 units per liter, most preferably 2,000 to 6,000 units per liter to obtain the "stone-washed" look. In a preferred mode the newly sewn jeans can be desized at 150° F. for 10 minutes, rinsed, contacted with about 1,000 to 6,000 CMC u/l of enzyme for 45 minutes at 160° F. while tumbling the jeans, washed, rinsed, softened and dried. A preferred method is as follows:

| Step           | Time    | Tempera-ture       | Machine Water Level | Product                | 15 |
|----------------|---------|--------------------|---------------------|------------------------|----|
| Shakeout       | 1 min.  | 150° F.            | 30"                 | Desizer                |    |
| Desize, stand. |         |                    |                     |                        |    |
| Rotation       | 10 min. | 150° F.            | 30"                 | Desizer                | 20 |
| Drain          | 3 min   | 150° F.            | 30"                 |                        |    |
| Rinse          |         |                    |                     |                        |    |
| Drain          | 45 min. | 160° F.            | 6"                  | Enzyme at 2000 CMC U/L |    |
| Abrade         |         |                    |                     |                        |    |
| Drain          | 2 min   | 150° F.            | 25"                 | —                      |    |
| Rinse          |         |                    |                     |                        |    |
| Drain          | 5 min   | 130° F.            | 12"                 | Bleach                 | 25 |
| Wash           |         |                    |                     |                        |    |
| Drain          | 3 min.  | 110° F.            | 22"                 | —                      |    |
| Rinse          |         |                    |                     |                        |    |
| Drain          | 3 min.  | 110° F.            | 22"                 | —                      |    |
| Rinse          |         |                    |                     |                        |    |
| Drain          | 5 min.  | 100° F.            | 12"                 |                        | 30 |
| Sour/Soft      |         |                    |                     |                        |    |
| Drain          | 4 min.  |                    |                     |                        |    |
| EXTRACT        |         |                    |                     |                        |    |
| TOTAL TIME     | 70 min. | (30 second drains) |                     |                        | 35 |

The treatment solutions used to contact the clothes can typically have the following ingredients.

TABLE 1

| Ingredient | Aqueous Treating Compositions |              |                |
|------------|-------------------------------|--------------|----------------|
|            | Useful                        | Preferred    | Most Preferred |
| Cellulase  | >1,000                        | 2,500-30,000 | 6,000-20,000   |
| Enzyme*    | —                             | 0.5-3        | 0.75-2.5       |
| Cellulase  | 0-1,000 ppm                   | 10-900 ppm   | 15-750 ppm     |
| Enzyme**   | 1-10                          | 2-8 l/gram   | 2-4 m l/gram   |
| Surfactant |                               |              |                |
| Aqueous*** |                               |              |                |
| treatment  |                               |              |                |

\*Amounts in CMC units per liter.

\*\*Lb. of enzyme/100 lbs. of fabric.

\*\*\*Amounts in ml of aqueous treatment per gram of fabric.

TABLE 2

| Ingredient | Concentrate Compositions |           |                |
|------------|--------------------------|-----------|----------------|
|            | Useful                   | Preferred | Most Preferred |
| Cellulase  | 1-90 wt %                | 2-80 wt % | 5-75 wt %      |
| Enzyme     | 99-0 wt %                | 98-5 wt % | 95-10 wt %     |
| Surfactant | Balance                  | Balance   | Balance        |
| Solvent    |                          |           |                |

TABLE 3

| Ingredient                              | Inorganic Solid Concentrate |            |                |
|-----------------------------------------|-----------------------------|------------|----------------|
|                                         | Useful                      | Preferred  | Most Preferred |
| Cellulase                               | 25-90 wt %                  | 30-85 wt % | 35-80 wt %     |
| Enzyme                                  | 20-60 wt %                  | 20-55 wt % | 25-50 wt %     |
| Hydratable Inorganic Salt Buffer System |                             |            |                |
| Sequestrant                             | 0-25 wt %                   | 5-20 wt %  | 7-15 wt %      |

TABLE 3-continued

| Ingredient         | Inorganic Solid Concentrate |           |                |
|--------------------|-----------------------------|-----------|----------------|
|                    | Useful                      | Preferred | Most Preferred |
| Water of Hydration | Balance                     | Balance   | Balance        |

TABLE 4

| Ingredient    | Organic Solid Concentrate |            |                |
|---------------|---------------------------|------------|----------------|
|               | Useful                    | Preferred  | Most Preferred |
| Cellulase     | 25-90 wt %                | 30-85 wt % | 35-80 wt %     |
| Enzyme        | 99-0 wt %                 | 98-5 wt %  | 95-10 wt %     |
| Surfactant    | 20-60 wt %                | 20-55 wt % | 25-50 wt %     |
| Sequestrant   | 0-25 wt %                 | 5-20 wt %  | 7-20 wt %      |
| Buffer System | 0-5 wt %                  | 1-4 wt %   | 1.5-3.5 wt %   |

\* PEG = polyethylene oxide (M.W. 1,000-9,000).

TABLE 5

| Ingredient           | Gelled Treatment Concentrate |  |
|----------------------|------------------------------|--|
|                      | Wt %                         |  |
| Liquid Enzyme        | 48%                          |  |
| Monosodium phosphate | 25.57%                       |  |
| Disodium phosphate   | 14.43%                       |  |
| Xanthan gum          | 0.48%                        |  |
| Water                | 11.52%                       |  |

TABLE 6

| Ingredient     | Liquid Concentrate |  |
|----------------|--------------------|--|
|                | Wt %               |  |
| Liquid enzyme  | 70.0%              |  |
| Sodium acetate | 28.59%             |  |
| Acetic acid    | 1.41%              |  |

TABLE 7

| Ingredient                | Liquid Enzyme Product Analysis |  |
|---------------------------|--------------------------------|--|
|                           | Wt %                           |  |
| Solids                    | 27.9%                          |  |
| Propylene glycol          | 24.0%                          |  |
| Sorbitol                  | 4.3                            |  |
| Alkali metal              | 0.3                            |  |
| Water                     | 48.1                           |  |
| pH of 1% aqueous solution | 6.6                            |  |
| Enzyme activity           | 1,000 CMC U/G                  |  |

TABLE 8

| Ingredient                | Liquid Enzyme Product Analysis |  |
|---------------------------|--------------------------------|--|
|                           | Wt %                           |  |
| Solids                    | 49.2                           |  |
| Sorbitol                  | 21.5                           |  |
| Alkali metal              | 1.9                            |  |
| Phosphorous               | 0.2                            |  |
| Water                     | 50.8                           |  |
| pH of 1% aqueous solution | 5.7                            |  |
| Enzyme activity           | 1,600 CMC U/G                  |  |

Tables 5-8 disclose useful gelled and liquid enzyme compositions that can be used in obtaining the "stone washed" look. The liquid enzyme products used in Tables 5 and 6 are set forth in Table 7.

The liquid concentrate compositions of this invention can be formulated in commonly available industrial mixers. Typically a solution of the surfactant is prepared in the solvent and into the surfactant solution is added the cellulase enzyme sufficiently slowly to create a uniform enzyme dispersion in the solvent. The con-

centrates can be packaged in typical inert packaging such as glass, polyethylene or polypropylene, or PET. Care should be taken such that agitation does not significantly reduce the activity of the cellulase enzyme.

The inorganic solid concentrate compositions of this invention can be made by combining the cellulase enzyme with the inorganic (alkali metal or alkaline earth metal) hydratable carbonate, bicarbonate, silicate or sulfate in an aqueous slurry containing sufficient water to cause the hydration and solidification of the inorganic components. The slurries can be made at elevated temperatures to reduce viscosity and increase handleability. The inorganic slurry compositions can then be cast in molds and after solidification can be removed from the mold, packaged and sold. Alternatively, the materials can be cast in reusable or disposable containers, capped and sold. Such materials usually are manufactured in a 1 ounce to 10 pound size. Solid concentrates can be in the form of a pellet having a weight of 1 gram to 250 grams, preferably 2 grams to 150 grams. The large cast object can be about 300 grams to 5 kilograms, preferably 500 grams to 4 kilograms.

The organic enzyme concentrate compositions can typically be made by slurring the enzyme material in a melted polymer matrix that can contain water for viscosity control purposes. Once a uniform dispersion of the enzyme, and other optional ingredients, are included in the organic polymer matrix, the materials can be introduced into molds or reusable or disposable containers, cooled, solidified and sold. Alternatively both the organic and inorganic solid concentrates can be made by combining the ingredients, and forming the compositions into pellets in commercially available pelletizing machines using either the temperature solidification, the hydration solidification mechanism, or a compression pelletizing machine using a binding agent well known in the art. All of the liquid and solid concentrate compositions of the invention can include additional ingredients that preserve or enhance the enzyme activity in the pumice-free stone wash processes of the invention.

The compositions of this invention are typically diluted in water in household, institutional, or industrial machines having a circular drum held in a horizontal or vertical mode in order to produce the "stone-washed" appearance without the use of pumice or other particulate abrasive. Most commonly the denim or other fabric clothing items are added to the machine according to the machine capacity per the manufacturer's instructions. Typically the clothes are added prior to introducing water into the drum but the clothes can be added to water in the machine or to the pre-diluted treatment composition. The clothing is contacted with the treatment composition and agitated in the machine for a sufficient period to ensure that the clothing has been fully wetted by the treatment composition and to ensure that the cellulase enzyme has had an opportunity to cleave cellulose in the fabric material. At this time if the treatment composition is to be reused, it is often drained from the tub and saved for recycle. If the treatment composition is not to be reused, it can remain on the clothing for as long as needed to produce color variation. Such treatment periods are greater than 5 minutes, greater than 30 minutes and up to 720 minutes, depending on amount of enzyme, during all or part of the mechanical machine action used to produce in the cellulase treated fabric the variations in color density. We believe that there is an interaction between the cellulase modi-

fied fabric and mechanical tumbling or action which removes cellulose from the fabric surface and the indigo dye to create a variation in color density from place to place on fabric panels and seams. Further, the action of the enzyme appears to cause puckering in the seams and a creation of a soft, wrinkled look in fabric panels.

The above specification provides a discussion of the compositions of the invention and methods of making and using the compositions in the "stone-washing" of fabric clothing items. The following Examples provide specific details with respect to the compositions and methods of the invention and include a best mode.

### EXAMPLES I-III

Into a Milnor 35 lb. capacity washing machine was placed new blue denim jeans and into the machine was placed 25 gallons of 120° F. water containing an amylase enzyme desizing stripper composition. The contents of the machine was agitated for 9 minutes and the aqueous solution was dumped. Into the machine was placed 17 gallons of water at 120° F. containing an amount of cellulase enzyme (see Table 5 below) and 10 milliliters of a sour comprising an aqueous solution containing 23 wt-% H<sub>2</sub>SiF<sub>6</sub> and 50 wt-% citric acid. The jeans were agitated in the cellulzyme composition for 1 hour and the aqueous composition was dumped. The jeans were then rinsed in three successive water rinses at 120° F., 110° F., and a final rinse at 100° F. containing 80 milliliters of softening agent and 5 milliliters of the sour product.

TABLE 9

| Example | Concen-<br>trate<br>Grams | CMCU/L* | CMCU/<br>LB* | CMCU/<br>Pair | Grams/<br>Pair |
|---------|---------------------------|---------|--------------|---------------|----------------|
| I       | 200                       | 7,459   | 32,000       | 48,000        | 20             |
| II      | 300                       | 11,189  | 48,000       | 72,000        | 30             |
| III     | 400                       | 14,918  | 64,000       | 96,000        | 40             |

\*Carboxymethyl cellulose units

TABLE 10

| Visible Spectrophotometer Scan of<br>Stone Washed Jeans and Product of Example II |                       |            |             |
|-----------------------------------------------------------------------------------|-----------------------|------------|-------------|
| Wave<br>Length                                                                    | Stone<br>Washed Jeans | Example II | Differences |
| 380                                                                               | 11.50                 | 11.01      | -0.49       |
| 390                                                                               | 15.71                 | 15.32      | -0.39       |
| 400                                                                               | 18.57                 | 18.49      | -0.08       |
| 410                                                                               | 21.70                 | 21.99      | 0.69        |
| 420                                                                               | 23.01                 | 24.22      | 1.20        |
| 430                                                                               | 22.96                 | 24.24      | 1.28        |
| 440                                                                               | 22.19                 | 23.53      | 1.34        |
| 450                                                                               | 21.31                 | 22.62      | 1.31        |
| 460                                                                               | 20.38                 | 21.64      | 1.26        |
| 470                                                                               | 19.43                 | 20.63      | 1.20        |
| 480                                                                               | 18.60                 | 19.71      | 1.10        |
| 490                                                                               | 17.91                 | 18.92      | 1.01        |
| 500                                                                               | 17.18                 | 18.08      | 0.90        |
| 510                                                                               | 16.35                 | 17.13      | 0.77        |
| 520                                                                               | 15.40                 | 16.06      | 0.66        |
| 530                                                                               | 14.40                 | 14.92      | 0.52        |
| 540                                                                               | 13.47                 | 13.88      | 0.41        |
| 550                                                                               | 12.77                 | 13.08      | 0.31        |
| 560                                                                               | 12.32                 | 12.60      | 0.28        |
| 570                                                                               | 11.94                 | 12.15      | 0.21        |
| 580                                                                               | 11.42                 | 11.59      | 0.17        |
| 590                                                                               | 10.85                 | 10.97      | 0.12        |
| 600                                                                               | 10.35                 | 10.39      | 0.04        |
| 610                                                                               | 9.95                  | 9.94       | -0.01       |
| 620                                                                               | 9.60                  | 9.56       | -0.04       |
| 630                                                                               | 9.15                  | 9.07       | -0.08       |
| 640                                                                               | 8.75                  | 8.64       | -0.11       |
| 650                                                                               | 8.44                  | 8.30       | -0.14       |
| 660                                                                               | 8.35                  | 8.21       | -0.14       |

TABLE 10-continued

| Visible Spectrophotometer Scan of<br>Stone Washed Jeans and Product of Example II |                       |            |             |
|-----------------------------------------------------------------------------------|-----------------------|------------|-------------|
| Wave<br>Length                                                                    | Stone<br>Washed Jeans | Example II | Differences |
| 670                                                                               | 8.66                  | 8.58       | -0.08       |
| 680                                                                               | 9.70                  | 9.73       | 0.03        |
| 690                                                                               | 11.83                 | 12.12      | 0.29        |
| 700                                                                               | 15.83                 | 16.60      | 0.77        |
| 710                                                                               | 22.62                 | 23.99      | 1.37        |
| 720                                                                               | 32.13                 | 33.84      | 1.71        |
| 730                                                                               | 42.55                 | 43.96      | 1.41        |
| 740                                                                               | 51.26                 | 51.92      | 0.65        |
| 750                                                                               | 57.04                 | 57.03      | -0.01       |

## DETAILED DISCUSSION OF THE DRAWINGS

FIG. 1 is a graphical representation of the data in the above table. The graph appears to be a single line consisting of dots and dashes, however the graph shows that the percent reflectance of the stone washed denims and the denims produced using the compositions and methods of this invention are virtually identical. The differences shown in column 4 of the above table indicate that at certain wavelengths minor differences occur, however the curves are virtually superimposable.

The above disclosure, Examples and data provide a complete discussion of the invention. However since many embodiments of the invention can be made without departing from the spirit and scope of the invention, the invention resides in the claims hereinafter appended.

I claim:

1. A gelled concentrate composition that can be used in aqueous solution to introduce, into the surface of dyed cellulosic fabrics, local areas of variations in color density, which consists essentially of:
  - (a) about 25-90 wt-% of a cellulase enzyme;
  - (b) about 0.01-10 wt-% of a thickener selected from the group consisting of a hydratable alkali metal or alkaline earth metal inorganic salt, a polyethylene oxide polymer, a polypropylene oxide polymer, a polyvinyl alcohol polymer, a polyvinyl pyrrolidone polymer, a polyalkyloxazoline polymer, a xanthum gum and mixtures thereof;
  - (c) about 0.1-50 wt-% of a buffer than can maintain the pH of the aqueous solution to about the optimum pH for enzyme activity;

wherein the variation in color density is substantially the same as that produced by conventional pumice stone processing.

2. The composition of claim 1 wherein the cellulase is a fungal cellulase.
3. The composition of claim 1 which additional contains an anti-redeposition agent.
4. The composition of claim 1 wherein the composition additionally contains an anti-foaming agent.
5. A liquid concentrate composition that can be used in aqueous solution to introduce, into the surface of dyed cellulosic fabric, local areas of variation and color density which consists essentially of:
  - (a) at least 25 wt-% of cellulase enzyme that can provide to an aqueous treatment solution at least 1,500 CMC units of enzyme per liter of solution;
  - (b) a alcoholic diluent selected from the group consisting of methanol, ethanol, isopropanol, tertiary butanol, ethylene glycol, propylene glycol, oligomers of ethylene glycol or propylene glycol and mixtures thereof; and
  - (c) a buffer that can maintain the pH of the aqueous solution at about the cellulase enzyme optimum pH;
- 25 wherein the variation in color density is substantially the same as that produced by conventional pumice stone processing.
6. A method of introducing into the surface of dyed cellulosic fabrics, localized area of variation and color density, which method comprises contacting the fabric with an aqueous composition consisting essentially of:
  - (a) a major proportion of water;
  - (b) at least 25 wt-% of a cellulase enzyme and at least 1,500 CMC units of cellulase enzyme per liter of aqueous composition; and
  - (c) a buffer that can maintain the pH of the aqueous solution at about the cellulase enzyme optimum pH;
- 35 wherein the fabric is contacted with the aqueous composition at a ratio of about 2-8 milliliters of aqueous solution per gram of dyed cellulosic fabric, and wherein the variation in color density is substantially the same as that produced by conventional pumice stone processing.
- 40
- 45 7. The method of claim 6 wherein the fabric is contacted with the aqueous solution for at least 5 minutes.
8. The method of claim 6 wherein the cellulase is a fungal cellulase.
9. The method of claim 6 wherein the fabric is indigo dyed denim.

\* \* \* \* \*